

## UNITED STATES PATENT OFFICE

2,361,805

## LUBRICATING COMPOSITION

Chester E. Wilson, San Pedro, Calif., assignor to  
Union Oil Company of California, Los Angeles,  
Calif., a corporation of California

No Drawing. Application April 11, 1942,  
Serial No. 438,649

20 Claims. (Cl. 252—53)

This invention relates to mineral lubricating oils modified by the addition of constituents capable of imparting to the oils characteristics adapting them especially to severe service uses such as are encountered in Diesel engines, high output aviation engines and the like. This application is a continuation in part of my earlier applications Ser. No. 305,496 filed November 21, 1939 and Ser. No. 345,844 filed July 16, 1940.

In severe service internal combustion engines, the operating conditions tend to cause the deposition of resinous and varnish-like products upon the pistons and around the rings to form lacquer-like coatings and deposits which tend to cause ring sticking and similar objectionable effects. In addition, there is a tendency to develop in the oil during use conditions which are corrosive to highly corrosion-sensitive bearings of the copper-lead and cadmium-silver type.

The principle object of this invention is to produce a lubricating oil which will have sufficient detergent properties to avoid the deposition of said resinous and lacquer-like materials, whereby to overcome ring sticking, valve sticking and the like, and which will at the same time prevent or overcome the development of corrosive conditions in the oil during use in internal combustion engines of said severe service types whereby to avoid objectionable corrosion of bearings of said copper-lead and cadmium-silver type.

Primarily the present invention resides in mineral lubricating oils which contain minor proportions of "oil-soluble" detergent soaps or salts, and minor proportions of "oil-soluble" "anti-corrosion" agents which will inhibit or control or overcome the development of conditions corrosive to said highly corrosion-sensitive bearings, said anti-corrosion agent being a condensation product of a phenol with an alcohol of sufficiently high order to impart good oil-solubility to the condensation product. Said anti-corrosion agent also serves to activate or in some manner to increase materially the detergent properties of the detergent soap or salt. The effects of the two agents used together are much greater than the additive effects of the same two agents used separately, and the result is the practical elimination of objectionable bearing corrosion described. The detergent soap or salt of this invention is a product of acidic materials obtained from petroleum, especially oil-soluble metal soaps or salts of synthetic acids derived from the oxidation of petroleum fractions, particularly by the oxidation of highly

paraffinic mineral lubricating oil fractions such as are described in the Bray Patent No. 2,270,620. Another form of detergent material may be a metal soap or salt of sulphonic acid derived from the well-known sulphuric acid treatment of mineral lubricating oil fractions such as those commonly known as "mahogany acids" from which the salts are prepared. Similarly oil-soluble naphthenates may be used.

10 A particular alcohol-phenolic condensation product to be used as an "anti-corrosion" agent is the product of condensation of stearyl alcohol with phenol in the presence of sulfuric acid as a catalyst.

15 As the terms are used herein, "oil-soluble" refers to a high state of colloidal dispersion of the soaps or salts in question, such that they maintain themselves permanently dispersed in the oil so as to approach a state of true solution.

20 The term "anti-corrosion" refers to the properties of the materials to neutralize synthetic acidity developed in the lubricating oil during use, or to inhibit oxidation or catalytic activity or the like, or otherwise control conditions which 25 would result in corrosive conditions. The term "detergent" refers to the property of an additive either to remove deposits of resinous and kindred materials from rings and grooves of piston and piston skirts, or to prevent such deposits, or to prevent formation and deposit in internal combustion engines.

30 The term "viscosity index" (V. I.) is an indication of the type of oil. A paraffin base oil is assigned the V. I. of 100 and a certain Gulf 35 Coast naphthenic oil has been assigned the V. I. of zero. High V. I. oils therefore are the so-called highly "paraffinic" oils such as Pennsylvania oils and those highly refined with selective solvents.

40 The term "soap" indicates those metal salts of high molecular weight acidic materials possessing enough carbon atoms, probably at least about ten carbon atoms, per molecule to impart good dispersibility or "solubility" in the mineral lubricating oil employed.

45 In practicing the invention, the particular type of detergent soap mentioned as being the metal salt of synthetic acids produced by the oxidation of mineral oil fractions may be obtained by the oxidation of said mineral oil fractions by procedures now well known. A preferable starting material is mineral lubricating oil of the so-called highly "paraffinic" nature such as that 50 obtained from Pennsylvania type oils, either

with or without the modern selective solvent treatment, and that obtained from Western or other mixed-base stocks containing paraffin base materials by the more modern highly selective solvent treatment with solvents such as phenol, furfural, liquid sulfur dioxide-benzene mixtures, dichlorethyl ether and the like. The oxidation is carried on to yield synthetic petroleum acids which are carboxylic acids, any preferred procedure for the production of these acids being employed.

The metal salts or soaps may be produced either by recovery of the acidics from the oils in any known or preferred manner or form, followed by production of the desired salt with an appropriate base, e. g. lime to produce calcium salts, or by the neutralization of the entire oxidized batch to produce the corresponding metal salts in situ in the unoxidized portions of the oil.

The sulfonic acids mentioned may be produced by any common method of producing petroleum sulfonic acids, such as treatment of a mineral lubricating oil fraction with fuming or concentrated sulphuric acid or chlorosulphonic acid. Commonly the so-called "mahogany acids" in solution in the unsulphonated oil are separated from the acid sludge containing the so-called "green acids" which are oil-insoluble. The sulphonate acid salts may be produced from the oil solution of sulphonic acids either by production of the desired salt in situ in the oil as by direct addition of the desired base, for example lime, or by conventional methods for recovering a sodium salt which may then be converted to other desired salts by metathesis. Again the sodium salt of such sulphonic acids is commonly obtainable on the market. However another form of sulphonate may be used which is prepared by sulphonating the oil to the desired extent, and then neutralizing the entire sulphonated batch with an appropriate base whereby green acid soaps formed are solubilized by the mahogany acid soaps with the result that both the green acid and the mahogany acid soaps go into solution in the oil to yield an acceptable oil concentrate of mixed green and mahogany sulphonates.

Ordinarily an alkaline earth metal will be used both for the sulphonates and for the oxidation acid salts, calcium salts being usually preferred. But heavy metal salts may sometimes be used, especially where the respective metal salts do not tend to increase corrosion conditions in use in the particular lubricating oil selected. Thus, aluminum and zinc salts are commonly acceptable, whereas in some lubricating oils iron and lead salts, and probably copper salts, are objectionable, especially in the sulfonates, because they tend to increase the development of corrosive conditions. However where there are only moderate tendencies of the metal salts to increase corrosive conditions in any given lubricating oil base, these may be adequately overcome by the presence of the anti-corrosion agent added according to this invention. This appears to be true of metals of salts of the oxidation acids and of the sulfonic acids.

Naphthenates may sometimes be employed, and when used the soaps or salts of those metals as above indicated will be employed which produce materials adequately soluble in the particular oil composition in the proportion required, e. g. 1% of aluminum or calcium naphthenate. Ordinarily the higher molecular weight acids produce soaps of greater oil-solubility, e. g.

75 naphthenates from lubricating oil treatment as distinguished from those from gas oil.

The anti-corrosion agent hereof is the condensation product of phenol with an alcohol of sufficiently high carbon content to insure that the phenolic product possesses good solubility in the oil employed. Thus, alcohols extending from about octyl alcohol or methyl cyclohexanol up through the scale including oleyl and stearyl alcohols and higher may be employed. A particular alcohol employed has been stearyl alcohol. The method for the production of a phenol-stearyl alcohol condensation product is typical of the other phenol-aliphatic alcohol condensation products. In condensing phenol and stearyl alcohol, sulphuric acid has been employed as a catalyst to yield a compound believed to be para-stearyl-phenol. The same catalyst may be used with any other alcohol indicated. In this method suitable mol proportions of the phenol and the stearyl alcohol or other alcohol are employed with several volumes of concentrated sulphuric acid. These materials are allowed to react. The reaction temperature should be controlled in order to avoid undesired reactions which might, for example, yield olefins rather than the desired condensation product.

One method which has been used to produce the stearyl alcohol-phenol product follows.

30 One hundred grams of stearyl alcohol plus 100 grams of phenol were added to 1000 grams of 80%  $H_2SO_4$  at 180° F. with stirring. The temperature rose to 192° F. Stirring was continued for five minutes after which the mixture was 35 poured into water and the solid material filtered off. Shaking this with ether and NaOH solution caused the slightly soluble sodium salt to crystallize out (80 grams). Forty-eight grams of this salt was heated with hydrochloric acid. 40 Naphtha was added and the mixture boiled to remove water and HCl. The naphtha solution was filtered to remove the precipitated sodium chloride, and the product was allowed to crystallize from the filtrate. The crystals were filtered off and washed with petroleum ether and dried. They weighed 36 grams. In order to remove any traces of strong acids the product was heated with dilute ammonium hydroxide, filtered off, and recrystallized from naphtha. 45 50 This material melts at 143° F. to 146° F. (62-63° C.) and apparently is p-octadecyl phenol.

In some instances it is satisfactory to employ this condensation product itself as the anti-corrosion agent. In other instances it may be preferable to employ salts of this phenolic product, for example the calcium salt.

Thus, the calcium salt of the stearyl alcohol-phenol condensation product may be prepared by agitating an oil solution of the condensation product with an equal mol proportion of hydrated lime at sufficiently elevated temperatures to cause reaction and formation of the desired calcium salt. Appropriate temperatures would be in the order of 200° F. or between about 175° F. and 225° F., for example. After reaction, the batch may be heated to around 300° F. for dehydration and then filtered or centrifuged to eliminate any solids. Apparently the formation of the salt may be facilitated by adding an approximately equal quantity of ethyl alcohol after the reaction is well under way, and continuing the reaction for an additional time, for example for another two hours following an initial two hours. Where alcohol is thus used there appears to be less hydrolysis and the calcium content

is increased. In removing solids and the like, a filter aid such as a ground diatomaceous earth may be employed. In the latter instance the batch will be heated, for example to 300° F., and filtered at that temperature while the viscosity of the liquid material is low.

In addition to lime salts or soaps of these phenolic condensation products, the other alkaline earth metal salts may be used. For some purposes it may also be satisfactory to employ salts of the heavy metals such as zinc, aluminum, nickel, copper, manganese, cobalt, iron, and the like. The principal consideration in the selection of the metal is that the product shall be adequately oil-soluble, and that under the existing conditions, and with the particular lubricating oil selected, the metal salts in the lubricating oil composition shall not act to increase the corrosion producing tendencies of the composition during use.

In selecting a lubricating oil, this may be a naphthenic base oil of any appropriate S. A. E. grade, or it may be an appropriate paraffinic base oil of high viscosity index where the additive materials have sufficient solubility in the oil. The sulfonates hereof are normally sufficiently soluble in the high viscosity index oils in the order of 90 V. I. to render them adaptable to use in such oils, whereas the synthetic acid salts are commonly more soluble in naphthenic base oils.

In compounding a lubricating oil containing these additives, the detergent soap, such as the calcium soap of the described synthetic acids produced by the oxidation of highly paraffinic mineral lubricating oil fractions, will be employed in an amount approximating 1%, for example 1.3%. The practical limits probably will be between about 0.4% or 0.5% and 2.5% or 3%. The same will be true of the sulphonates, and of naphthenates. The amounts used should be such as not to increase materially the viscosity of the base oil.

With respect to the phenol-alcohol condensation product, here also the percentage may be in the order of 1%, but commonly a somewhat smaller proportion may be employed, for example around 0.5% to 0.7%. Here the limits probably would range from about 0.1% to 2% or 3%. Commonly larger percentages do not greatly increase the effects derived from the materials and serve only to increase the cost, although sometimes it is found that greater proportions of the detergent salt, e. g. 2.5%, are desirable where there is no metal constituent in the anti-corrosion agent to increase the ash content. For example, where the detergent soap might be confined to 1.5%, if about 1% of an anti-corrosion agent is employed which contains a metal constituent, about 2.5% of the detergent salt has been satisfactorily used with an anti-corrosion agent containing no metal. This has been particularly true in employing sulphonates such as calcium sulphonate with a metal-free anti-corrosion agent.

In addition to the indicated straight chain alcohols to be used in preparing a phenol condensation product, I may use other saturated alcohols such as the cyclo-aliphatic alcohols with or without an aliphatic chain substituent. For example ethyl cyclo-hexanol may be used. Also I may employ the alcohols produced from naphthenic acids which are here termed naphthenyl alcohols. The naphthenes are commonly understood to consist of saturated five or six-carbon

5 rings substituted with aliphatic chains of greater or lesser length. In addition I may use other alcohols containing rings where the phenol condensation products, or the salts thereof, are sufficiently oil-soluble, such as benzyl alcohol.

In the above descriptions, the commonly known phenol  $C_6H_5OH$  has been intended. However other phenolics may be employed. Alkyl substituted phenols may be desirable where low molecular weight or polyhydroxy alcohols are used, it being the intent to include in the molecule an adequate number of carbons to insure good oil-solubility. However where substituted phenols are employed, it is necessary that not all positions be substituted, whereby to leave at least one reactive hydrogen for substitution of the alcohol constituent. Other phenols may include the plural ring compounds such as naphthols, pyrogallol and the like together with various alkyl substituted derivatives thereof as above indicated.

While the alcohols previously mentioned are monohydroxy alcohols, it is not necessary that the alcohols be so limited. Polyhydroxy alcohols may be used so long as the condensation product contains enough carbon atoms (probably at least about twelve carbons per each phenolic group) so as to render the material oil-soluble, such as glycerol or ethylene glycol. To obtain sufficient carbons such an alcohol may be condensed with an alkylated phenol, as may any other alcohol.

Metals for salts of these various condensation products will be those used for other salts as above described. Salts of all the phenolics described are, in general, deemed preferable to the phenolics themselves. Lubricating oils compounded as described will possess viscosities not substantially higher than those of the base lubricating oils employed.

40 Various modifications in the scope of the appended claims will be apparent to those skilled in the art.

I claim:

1. A lubricating oil comprising a mineral lubricating oil fraction, a minor proportion of oil-soluble metal soap of acids derived from petroleum, and a minor proportion of oil-soluble compound from the condensation of a phenol with an alcohol containing at least about eight carbon atoms per molecule.

2. An oil according to claim 1 wherein the alcohol is a monohydroxy alcohol.

3. An oil according to claim 1 wherein the alcohol is a straight chain alcohol.

4. An oil according to claim 1 wherein the alcohol is a polyhydroxy alcohol.

5. An oil according to claim 1 wherein the alcohol is aromatic.

6. An oil according to claim 1 wherein the alcohol is a cyclo-aliphatic alcohol.

7. A lubricating oil comprising a mineral lubricating oil fraction, a minor proportion of oil-soluble metal soap of synthetic acids produced by the oxidation of a petroleum fraction, and a minor proportion of oil-soluble compound from the reaction of a phenol with an alcohol containing at least about eight carbon atoms per molecule.

8. An oil according to claim 7 wherein the alcohol is a straight chain alcohol.

9. An oil according to claim 7 wherein the alcohol is a straight chain alcohol substituted with an aromatic ring.

10. An oil according to claim 7 wherein the alcohol is stearyl alcohol.

11. A lubricating oil comprising a mineral lubricating fraction containing a minor proportion of oil-soluble metal petroleum sulfonate and a minor proportion of oil-soluble product from the condensation of a phenol with an alcohol containing at least about eight carbon atoms per molecule.
12. An oil according to claim 11 wherein the alcohol is a straight chain alcohol.
13. An oil according to claim 11 wherein the alcohol contains a ring.
14. An oil according to claim 1 wherein the compound from the condensation is a metal salt of the condensation product.
15. An oil according to claim 1 wherein the compound from the condensation is an alkaline earth metal salt of the condensation product.
16. An oil according to claim 1 wherein the compound from the condensation is the calcium salt of the condensation product.
17. An oil according to claim 1 wherein the phenol is an alkylated phenol.
18. An oil according to claim 1 wherein each additive is present in the oil in an amount in the order of 1%.
19. An oil according to claim 1 wherein the petroleum acid salt is present in the order of a little more than 1% and the condensation compound is present in the order of a little less than 1%.
20. A lubricating oil comprising a mineral lubricating fraction containing a minor proportion of oil soluble metal soap of synthetic acids obtained from the oxidation of highly paraffinic lubricating oil fractions and a minor proportion of an oil soluble compound from the condensation of phenol with an alcohol containing at least about 8 carbon atoms per molecule.